

# UNITED STATES PATENT OFFICE

FRANK A. FAHRENWALD, OF CLEVELAND HEIGHTS, OHIO.

## APPARATUS FOR HIGH-TEMPERATURE USES.

1,357,549.

Specification of Letters Patent.

Patented Nov. 2, 1920.

No Drawing.

Application filed August 25, 1919. Serial No. 319,756.

To all whom it may concern:

Be it known that I, FRANK A. FAHRENWALD, a citizen of the United States, residing at Cleveland Heights, in the county of Cuyahoga and State of Ohio, have invented a certain new and useful Improvement in Apparatus for High-Temperature Uses, of which the following is a full, clear, and exact description.

10 This invention relates to alloys and has for its especial object the provision of an inexpensive and mechanically strong composition of matter which shall withstand repeated exposure to high temperatures without material oxidation, disintegration or change of shape. A great need exists for such an alloy in the manufacture of heat treating boxes; carbonizing boxes; lead pots; furnace parts; retorts for the distillation of wood, coal oil and oil bearing shales; containers for the production of calcium cyanamid; doors, chains, links and rabble arms for metallurgical furnaces; and many other metallurgical and chemical relations. 15

20 Also such alloys in case they have the requisite hardness are of great value for cutting tools and tools for working hot metal. All the foregoing uses are grouped under the expression "Apparatus for high temperature uses."

25

The essential desiderata of such apparatus are cheapness and availability, coupled with reasonably long life. Containers, boxes, and some other articles have been made from certain alloys of nickel and chromium, and serve very effectually the uses to which they are put but their expensiveness is absolutely prohibitive for most purposes, and the same is true of most other compositions heretofore proposed for such uses. 30 The object of my invention is to secure a sufficiently resistant alloy for most practical purposes with the use of inexpensive ingredients and without requiring expensive processes of manufacturing. My improved alloy may be either cast directly to shape or by suitable precautions in composition can be machined as hereafter set forth.

35 Although special substances may be added for special purposes as hereafter set forth my improved apparatus is ordinarily made from an alloy containing essentially the following ingredients, (the first column showing substantially the preferred compo-

sition and the second column the variations):

|           |       |           |
|-----------|-------|-----------|
| Iron      | 70%   | (55%-75%) |
| Chromium  | 15%   | (10%-20%) |
| Cobalt    | 13.5% | (10%-20%) |
| Manganese | .5%   | (.2%-1%)  |
| Silicon   | .5%   | (.2%-3%)  |
| Carbon    | .5%   | (.2%-3%)  |

The iron constitutes the base of the alloy and is chosen for its cheapness, its amount decreasing with the excellence of the composition, although preferably preponderant in all cases. The chromium affords resistance to oxidation at high temperatures and increases the solubility of the minor constituents thus improving the physical properties of the alloy. The cobalt is employed for its toughening and hardening qualities. Cobalt in an amount of 10% or greater has a hardening effect superior to that produced by any amount of nickel whatever. In quantities less than about 10% cobalt is not appreciably superior to nickel in this regard, and suffers the drawback that its price is about three times that of nickel, while above about 15% to 20% its hardening effect does not increase proportionally to the increased price consequent upon its use. The manganese is employed as a scavenger and to improve the casting qualities of the alloy. The silicon has a decided hardening effect and also the added quality of shielding other ingredients against oxidation although in its larger quantities it tends to produce brittleness which restricts its use. The carbon tends to produce hardness, increases the resistance of the alloy to deformation at points below fusion and also increases the fluidity of the molten alloy thus assisting in the casting. If the carbon and silicon are both restricted to .5% or less of the alloy, the articles cast therefrom can be readily machined after annealing.

The addition to the alloy of from about 1% to about 8% of a tungsten-like metal (by which I mean tungsten or molybdenum) greatly increases its resistance to distortion at high temperatures and so improves it for many uses as for example in tools for working hot metal.

No special precautions are required in the manufacture of the alloy since it can be made either in crucibles or by the electric

furnace method although I prefer to employ the method described and claimed in my application filed simultaneously herewith and denominated case E. The only precautions necessary are to restrict the carbon and silicon to the desired limits and this is peculiarly easy with my improved process although it can be accomplished in other ways. It is also necessary to restrict the 10 sulfur and phosphorus to less than about .05% each which can be effected by a proper selection of the ore coupled with the use of suitable slags and furnace linings as will be well understood by those skilled in the art 15 of iron metallurgy. It will also be understood that other ingredients can be added than those herein listed and generally that many variations in composition are permitted within the scope of the claims hereto annexed.

Having thus described my invention what I claim is:—

1. Apparatus for high temperature uses made from an alloy containing a preponderance of iron together with from about 10 to 25 20 per cent. of each of the metals cobalt and chromium, and at least about .2% of each of the substances—carbon, silicon, and manganese.

2. Apparatus for high temperature uses 30 made from an alloy containing from about 10 to about 20 per cent. of each of the metals cobalt and chromium, together with from about .2% to 3% of each of the substances carbon and silicon, the balance being mostly 35 iron.

3. Apparatus for high temperature uses made from an alloy containing a preponderance of iron alloyed with ten to twenty per cent. of cobalt and small amounts of carbon, 40 silicon, and manganese, the balance consisting essentially of one or more metals from the chromium group.

4. Apparatus for high temperature uses made from an alloy containing a preponderance 45 of iron together with about ten to twenty per cent. of each of the metals cobalt and chromium, and about one to eight per cent. of a tungsten-like metal, and also small amounts of carbon and silicon. 50

5. Apparatus for high temperature uses made from an alloy containing substantially iron 70%, chromium 15%, cobalt 13% to 55 14% and fractional percentages of carbon, silicon, and manganese.

In testimony whereof, I hereunto affix my signature.

FRANK A. FAHRENWALD.